

## UNITED STATES PATENT OFFICE.

FREDERICK J. READ, OF SAN FRANCISCO, CALIFORNIA, ASSIGNOR, BY DIRECT AND MESNE ASSIGNMENTS, OF ONE-HALF TO CALAVERAS IRON AND STEEL COMPANY, A CORPORATION OF NEVADA, AND ONE-HALF TO SYDNEY H. DEMAREST, OF SAN FRANCISCO, CALIFORNIA.

## METAL.

No Drawing.

Application filed September 28, 1927. Serial No. 222,687.

My invention relates to a metal made by the combination of several other metals and which is adapted for a variety of uses particularly in journals and bearings.

5 An object of my invention is to produce a metal which will have superior characteristics for use in bearings over metals at present available.

10 Another object of my invention is to utilize materials which are economically available to produce a new metal having superior characteristics.

15 The invention possesses other advantageous features, some of which with the foregoing, will be set forth at length in the following description where I shall outline in full the preferred form of my invention.

20 The metal of my invention preferably comprises an alloy including aluminum treated with cerium and combined with copper.

Although the metal produced by my invention is applicable to a wide variety of uses such as for electrical conductors, for commutators and in similar circumstances, it is 25 particularly adapted to be used as bearing metal for shafting which is subjected to severe service and heavy loads. The metal radiates heat rapidly from a journal so that relatively close clearances can be used and is 30 capable of running for protracted periods with a minimum amount of lubrication or no lubrication at all. Although the use to which the metal is to be put dictates somewhat the procedure utilized in preparing it, 35 I shall describe the general method to be followed in preparing my metal and particularly a manner which will produce an excellent metal for bearings.

40 The metal of my invention comprises in its make up a portion of cerium, and as a convenient and economical source of cerium I preferably utilize chalcopyrite, which as found in certain localities, has associated with it a sufficient amount of cerite to furnish the 45 necessary cerium and to justify its use in my process of producing the metal. Chalcopyrite contains a considerable proportion of iron which I do not desire to have present in appreciable quantities in my completed prod-

uct so that I first treat the chalcopyrite with 50 sulphuric acid, usually in aqueous solution and with the chalcopyrite in finely divided form so that practically all of the iron is removed. Other acids also can be used and other methods of extracting the iron but I 55 have found that sulphuric acid is advantageous.

In order to render the cerium effective upon the aluminum, I either immerse the metallic aluminum in the aqueous solution of treated chalcopyrite, as mentioned above, or I evaporate the aqueous solution to a dry powder and mix it with the aluminum in a crucible. In the final product, the aluminum, which preferably is of the grade and purity known 60 as virgin aluminum, ranges from 5 to 10 per cent and the cerium can vary between 1/16 of one per cent and 10 per cent dependent upon the desired characteristics of the metal. I 65 preferably utilize the treated chalcopyrite 70 and the treated aluminum in proportions to produce this result and add sufficient copper to the aluminum in the crucible to make up the necessary 100 per cent. The amount of copper is varied to compensate for impurities in the metal and for the varying percentage of aluminum and cerium. 75

When the treated aluminum or the aluminum and powder resulting from the treated chalcopyrite are placed in a crucible with 80 copper, they are heated until the aluminum and copper are fused and form an alloy. The cerium also enters into the combination so that when the fused metal has cooled there is produced an alloy of metal which is ready 85 to be reheated for casting and which has vastly superior characteristics over other metals for bearings and for other uses as mentioned above.

I claim:

90 A metal comprising an alloy including from one-tenth of one per cent to ten per cent cerium, from five to ten per cent aluminum, and substantially all of the remainder copper.

95 In testimony whereof, I have hereunto set my hand.

FREDERICK J. READ.